

## UNITED STATES PATENT OFFICE

2,589,951

PRINTING OF WOOLEN TEXTILES WITH A  
NONAQUEOUS PASTE COMPRISING A DYE-  
STUFF CONTAINING AN ACID GROUP, A  
WATER-INSOLUBLE VINYL POLYMER, AND  
AN ACID-LIBERATING AGENTErwin Meier, Neuewelt, near Basel, Switzerland,  
assignor to Ciba Limited, Basel, Switzerland, a  
Swiss firmNo Drawing. Application June 20, 1949, Serial  
No. 100,296. In Switzerland July 2, 1948

9 Claims. (Cl. 8—62)

1

The present invention relates to the printing of textiles.

In the normal printing of textiles, the usual procedure is to print the material to be printed with a printing paste which contains, in aqueous suspension or solution, a dyestuff which possesses sufficient affinity for the fiber to be colored. In this connection, the printing paste is brought into the consistency necessary for the printing, with the aid of an inert thickening agent. Conventionally, the dyestuff is fixed, after the printing and drying of the material, by a steaming process. Thereafter, the thickening agent has to be removed from the fiber by means of a rinsing or washing process, and there is finally obtained a sort of locally limited dyeing on the textile material which is employed. This method is capable of very wide application, but is bound up with the disadvantage that the printing operation requires various manipulations such as printing, drying, steaming, washing, repeated drying, etc., all of which have to be carried out in more or less close succession.

Printing processes have also been recommended wherein the dyestuff is fixed on the fiber with the aid of a binding agent.

In this type of process, the dyestuff which is employed need not have an affinity for the textile fiber, so that it is possible to use pigments and the like as the coloring material. However, it is very difficult, in such processes, to realize a sufficient adherence of the coloring matter to the fiber, without the incidence of a frequently undesirable stiffening of the printed places by means of the binding agent, so that, notwithstanding the simplicity of the printing procedure therein, this type of process has not found general acceptance. It is also to be noted that, in many processes of this character, it is necessary to effect a hardening of the binding agent at temperatures which are considerably higher than the usual drying temperatures and that, secondly, special heating chambers are required in order to successfully carry out such processes.

It has now been found that textile structures which are made, wholly or in part, of animal fibers or other fibers having similar dyeing properties, can be advantageously printed with dyestuffs which have affinity for these fibers, if use is made of a printing paste which, in addition to the dyestuff, contains a non-aqueous thickener which comprises a water-insoluble polymer as well as an agent which splits off acid.

As textile structures of the said type, use may be made more particularly of fabrics and knitted articles made of animal fibers or fibers which have a similar dyeing behavior, for example fab-

2

rics made of superpolyamides, or of silk, or particularly of wool. In connection with the use of wool, it is important that, in practicing the present invention, use may be made of chlorinated wool and also of unchlorinated wool.

The dyestuffs to be used according to the present invention must possess affinity for the fibers which are employed. As such, the so-called basic dyestuffs, for example, can be used. However, use may be made with advantage of dyestuffs with acid groups, for example acid dyestuffs such as are conventionally used for dyeing wool. Such acid dyestuffs may be monoazo and disazo dyestuffs which contain acid groups, such as carboxylic acid or sulfamide groups, especially however sulfonic acid groups, as well as dyestuffs of other classes, e. g. acid triarylmethane or anthraquinone dyestuffs. However, it is also possible to use, for the present process, as dyestuffs which contain acid groups, most so-called substantive dyestuffs which always contain acid groups and which are usually used for dyeing and printing cellulose fibers. Such substantive dyestuffs with acid groups are generally disazo or polyazo dyestuffs and may preferably contain sulfonic acid groups as the acid groups. In view of the non-aqueous character of the thickener, it is normally preferable to use dyestuffs which are soluble in the thickeners employed, or to use the dyestuffs in a form which is as free as possible of inorganic solids, i. e. in concentrated form, since otherwise defects due to insufficient solubility may be encountered. On the other hand, the dyestuffs may contain metals such as copper, cobalt, nickel, iron and, especially, chromium in complex combination.

The non-aqueous thickeners used for preparation of the printing pastes, may contain, as thickening agents, preferably water-insoluble vinyl polymers, especially polyvinyl acetate, polyvinyl chloride, as well as mixed acetate-chloride polymers, severally or in admixture with each other. Such thickening agents are soluble or swellable in many non-aqueous solvents or thickening agents, e. g. in cyclohexanone, butyl acetate, glycol monoalkyl ethers such as glycol monomethyl ether. In this connection, it is advantageous to select solvents, e. g. butyl acetate, which exert an appreciable softening action and/or to add softening agents, such as dibutyl phthalate.

Of particular significance to the present invention, is the addition to the non-aqueous thickener, of an agent which splits off acid when heated. The said agent may be any of the conventional agents of this kind, e. g. of the kind which liberates acid by dissociation of a salt or by saponification of an ester. In selecting the

agent which splits off acid, it is of course necessary to assure a certain compatibility with the non-aqueous thickener. Acid-liberating agents which naturally contain water or are naturally strongly hygroscopic may give rise to difficulties, but use may be made among others of ammonium tartrate, ammonium thiocyanate, and malonic acid diethyl ester, although ammonium chloride and ethyl tartrate are especially advantageous because of their good action and compatibility with the non-aqueous thickeners.

In the preparation of printing pastes, the quantity of dyestuff to be used naturally depends upon the dyeing strength which is desired to realize by the printing. The relative proportion of solvent and polymerizate used as thickener should be so selected that a paste is produced which can be printed with the usual printing apparatus. In determining the amount of acid-liberating agent to be added, it is to be noted that with increasing quantities of such agent, for example between about 20 and 60 grams of ethyl tartrate per kilogram of printing paste, the improving action is progressively increased, while with a further increase, e. g. between about 70 and 80 grams per kilogram of printing paste, a maximum is attained which is no more or at least not appreciably exceeded if the quantity of acid-liberating agent is further increased. When ammonium chloride is used, a quantity of 50 grams per kilogram generally suffices to give an optimum action, while greater amounts tend to give an undesirable gelation with many printing pastes.

The printing process, whereby textile material is printed with a paste according to the invention, is per se no part of the latter and any conventional process, such as hand printing or the like, may be employed. The material being printed may advantageously be wool muslin, but lighter fabrics and cheviot may also be used. While the usual printing processes are practically restricted to chlorinated wool, the present invention makes it possible to print unchlorinated wool also, without entailing any appreciable decrease in dye strength and brilliance.

Prints obtained according to the present invention may be used after drying, if desired, without being subjected to any aftertreatment, if the product will not be exposed to conditions which require wet fastness and fastness to rubbing. Such prints are advantageous in that they can be rolled up, after drying, and stored for long periods of time, and that their fastness properties are substantially improved when they are subjected to a steaming or setting treatment such as is usual in the conventional handling of wool, for example in decatizing wool. It may be that the acid-liberating agent functions during such treatment to effect a fixing of the dyestuff on the fiber, bringing the normal affinity of the dyestuff for the fiber into play. In any event, the appearance of such a fixing reaction is surprising since it would be expected that the dyestuff would be embedded in the water-insoluble thickening agent, and therefore could not come into reaction with the fiber. In comparison with the usual printing process with aqueous pastes, printing according to the present invention presents the advantage that it is unnecessary to remove the thickening agent, and in comparison with the aforementioned prior process wherein the dyestuff is fixed on the fiber by means of binding agents, the advantage that stiffening of the printed places may be avoided

without encountering poor fixation of the dyestuff. It is also possible, if desired, to effect fixation of the prints according to the invention by means of a normal steaming treatment directly following the printing. Of great importance is the fact that the otherwise necessary rinsing and washing treatment for the removal of the thickening agent is not necessary according to the present invention.

This makes it possible to use the present invention in many cases where hitherto no suitable printing process has been available. In many instances, the character of the material or of the area to be printed excluded any possibility of a washing treatment for the removal of the thickening agent, for example in the case of certain taffeta fabrics for children or jacquard decorating material made of natural silk or wool or mixed fabrics containing such fibers. In the case of jacquard fabric, a washing treatment displaces the fibers, while in the case of taffeta, creases and wrinkles are produced which can hardly be removed. With many unchlorinated wool fabrics and wool-mixed fabrics, there is also the difficulty that washing will cause undesired shrinking or that a yellowish coloration will develop on drying.

The following examples further illustrate the present invention, without however being at all limitative thereof. In such examples, the parts—unless otherwise indicated—are parts by weight, percentages are percentages by weight, and temperatures are in degrees centigrade.

#### Example 1

A printing paste, prepared by admixing the following:

10 parts of the dyestuff,  
300 parts of ethyl glycol,  
250 parts of cyclohexanone,  
150 parts of dibutyl phthalate,  
60 parts of butyl acetate,  
50 parts of a solution which contains, per 100 parts, 54 parts of acetone, 4 parts of butyl acetate, 20 parts of tricresyl phosphate, 6 parts of polyvinyl acetate-chloride mixed polymer and 16 parts of alcohol-moistened nitrocellulose,  
80 parts of polyvinyl chloride,  
100 parts of ethyl tartrate.

1000 parts

is homogenized in a wet-dye mill. The paste is used for printing on wool muslin, which is then dried and treated for ten minutes in a Mather-Platt apparatus.

#### Example 2

The printing paste of Example 1 is replaced by a paste made of the following ingredients:

10 parts of dyestuff,  
100 parts of ethyl glycol,  
355 parts of cyclohexanone,  
110 parts of dibutyl phthalate,  
210 parts of butyl acetate,  
50 parts of a solution which contains, per 100 parts, 54 parts of acetone, 4 parts of butyl acetate, 20 parts of tricresyl phosphate, 6 parts of polyvinyl acetate-chloride mixed polymer and 16 parts of alcohol-moistened nitrocellulose,  
65 parts of polyvinyl chloride,  
100 parts of ethyl tartrate.

1000 parts

**5**  
*Example 3*

Chlorinated wool muslin is printed with a printing paste of the following composition:

10 parts of dyestuff,  
125 parts of ethyl glycol,  
300 parts of cyclohexanone,  
100 parts of dibutyl phthalate,  
250 parts of butyl acetate,  
50 parts of solution (as in preceding examples),  
65 parts of polyvinyl chloride,  
100 parts of ethyl tartrate.

1000 parts

Fixing is effected by decatizing the wool on a hot-pressing machine.

The indicated paste may be replaced by any one of the following pastes:

| Printing Paste       | Parts by Weight— |       |       |
|----------------------|------------------|-------|-------|
|                      | 1                | 2     | 3     |
| Dyestuff             | 10               | 10    | 10    |
| Ethyl Glycol         | 125              | 125   | 280   |
| Cyclohexanone        | 300              | 300   | 300   |
| Dibutyl Phthalate    | 100              | 100   | 100   |
| Butyl Acetate        | 250              | 250   | 130   |
| Solution (as above)  | 50               | 50    | 50    |
| Polyvinyl Chloride   | 65               | 65    | 65    |
| Ammonium Tartrate    | 100              | 100   | —     |
| Ammonium Thiocyanate | —                | —     | —     |
| Ammonium Chloride    | —                | —     | 65    |
| Total                | 1,000            | 1,000 | 1,000 |

In each case, the chlorinated wool may be replaced by unchlorinated wool muslin, light wool cloth or cheviot.

*Example 4*

Chlorinated wool fabric is printed with a printing paste of the following composition:

10 parts of dyestuff,  
300 parts of ethyl glycol,  
300 parts of cyclohexanone,  
100 parts of dibutyl phthalate,  
75 parts of butyl acetate,  
40 parts of acetone,  
10 parts of alcohol-moistened nitrocellulose,  
65 parts of polyvinyl chloride,  
100 parts of ethyl tartrate.

1000 parts

The printed fabric may be hot-pressed or steamed, whereupon the acid-eliminating agent is activated and the dyestuff is fixed.

In lieu of chlorinated wool fabric, use may also be made of the unchlorinated material. The ethyl tartrate may be replaced by 50 parts of ammonium chloride, in which case the butyl acetate may be increased to 125 parts.

In the foregoing embodiments, the printing pastes always contain a small quantity of nitrocellulose. It is to be understood, however, that this is not absolutely necessary to the invention; however, the nitrocellulose tends to counteract the adhesiveness of the print made on the polyvinyl resin basis and is therefore advantageously included. If desired, the nitrocellulose may be replaced by acetyl cellulose or other similar compound.

As the dyestuff in the preceding examples, use may be made inter alia of any of the following.

**6**

Colour Index  
No.

1. Rhodamin G. extra----- 750
2. Victoria Blue B----- 729
- 5 3. Spirit Black CL----- 864
4. Brilliant Glacier Blue----- 664
5. Auramin O----- 655
6. Eosin DWC----- 768
7. Rhodamin B extra----- 749
- 10 8. Copper compound of the dyestuff of the formula



- (green)
9. Dyestuff from diazobenzene and 1-(2'-chloro-5'-sulfophenyl)-pyrazolone - 3 - carboxylic acid (yellow);
10. Dyestuff from diazobenzene and 1-(2'-chloro-5'-sulfophenyl) - 3-methylpyrazolone (yellow);
11. Chromium compound of the dyestuff from 2-diazo-1-hydroxy-4-nitrobenzene - 6 - sulfonic acid and acetic acid anilide (yellow);
12. Chromium compound of the dyestuff from 2-diazo-1-hydroxy-4-nitrobenzene - 6 - sulfonic acid and 1-phenyl-1-methyl-pyrazolone (orange);
13. Chromium compound of the dyestuff from 2-diazo-1-hydroxybenzene-4-sulfamide and 1-(3'-sulfamidophenyl)-3 - methyl - pyrazolone (orange);
14. Chromium compound of the dyestuff from 2-diazo-1-hydroxy - 4 - chlorobenzene-6-sulfonic acid and 1-phenyl-3-methyl-pyrazolone (orange);
15. Cobalt compound of the dyestuff from 2-diazo-1-hydroxybenzene-4-sulfamide and 2-hydroxynaphthalene (red);
16. Chromium compound of the dyestuff from 1-diazo-2-hydroxynaphthalene - 4 - sulfonic acid and 1-phenyl-3-methyl-pyrazolone (red);
- 55 17. Dyestuff of the formula



- 70 18. Dyestuff obtained by condensation of 1 mol of cyanuric acid chloride with 1 mol of 1-amino - 4 - (4'-aminophenyl) - aminoanthraquinone-2,3'-disulfonic acid, 1 mol of 4-amino-4'-hydroxy-1,1'-azobenzene-3' - carboxylic acid and 1 mol of aniline (blue);

19. Condensation product from 2 mols dehydrothio-p-toluidine-monosulfonic acid and 1 mol of 4,4'-dinitrostilbene-2,2'-disulfonic acid with subsequent oxidation with hypochlorite (yellow).

Having thus disclosed the invention, what is claimed is:

1. In a process for printing a textile structure of wool with a dyestuff containing an acid group, the improvement which consists of applying the said dyestuff with the aid of a printing paste including a non-aqueous thickener containing a water-insoluble vinyl polymer and an acid liberating agent.

2. In a process for printing a wool fabric with a dyestuff containing an acid group, the improvement which consists of applying the said dyestuff with the aid of a printing paste including a non-aqueous thickener containing polyvinyl chloride and an acid-liberating agent, and then steaming the printed product.

3. A non-aqueous printing paste containing, as special assistants, a water-insoluble vinyl polymer and an acid-liberating agent, in addition to a dyestuff having affinity for animal fibers.

4. A non-aqueous printing paste containing an acid dyestuff and a non-aqueous thickener containing a water-insoluble vinyl polymer and an acid-liberating agent.

5. A non-aqueous printing paste containing a substantive dyestuff and a non-aqueous thickener containing a water-insoluble vinyl polymer and an acid-liberating agent.

6. A non-aqueous printing paste containing an acid dye-stuff and a non-aqueous thickener containing a water-insoluble vinyl polymer, a softening agent and an acid-liberating agent.

7. A non-aqueous printing paste containing a substantive dyestuff and a non-aqueous thickener containing a water-insoluble vinyl polymer, a softening agent and an acid-liberating agent.

8. A non-aqueous printing paste containing an acid dyestuff and a non-aqueous thickener containing polyvinyl chloride and ethyl tartrate as acid-liberating compound.

9. A non-aqueous printing paste containing an acid dyestuff and a non-aqueous thickener containing polyvinyl chloride and ammonium chloride as acid-liberating compound.

ERWIN MEIER.

#### REFERENCES CITED

The following references are of record in the file of this patent:

#### UNITED STATES PATENTS

| Number    | Name        | Date          |
|-----------|-------------|---------------|
| 1,787,239 | Fleischmann | Dec. 30, 1930 |
| 2,052,000 | Oschatz     | Aug. 25, 1936 |

#### FOREIGN PATENTS

| Number  | Country       | Date          |
|---------|---------------|---------------|
| 589,020 | Great Britain | June 10, 1947 |